

# UNITED STATES PATENT OFFICE.

WILLIAM N. BLAKEMAN, JR., OF MOUNT VERNON, NEW YORK.

## PAINT VEHICLE FOR ANHYDROUS PIGMENTS.

1,385,033.

Specification of Letters Patent. Patented July 19, 1921.

No Drawing.

Application filed June 12, 1917. Serial No. 174,255.

To all whom it may concern:

Be it known that I, WILLIAM N. BLAKEMAN, Jr., a citizen of the United States, and resident of the city of Mount Vernon, in the 5 county of Westchester and State of New York, have invented a new and useful Paint Vehicle for Anhydrous Pigments, which invention is fully set forth in the following specification.

10. The object of this invention is to utilize as pigments, in the art of painting, in an economical and satisfactory manner, all matter that is stable in character, and can be reduced to an amorphous and impalpable condition.

15. The behavior of pigments toward oil-vehicles, when ground therein, is by no means uniform, very many of the combinations thus made, especially those with anhydrous 20 pigments, showing an utter lack of spreading power and diffusive opacity; and these marked deficiencies greatly detract from their usefulness.

25. I have discovered that all pigments may be ground with an agent that will harmonize and combine with them, and that the magma so formed will also be congruent to and combine with all oil-vehicles and possess, when ground therein, great spreading power, 30 accelerated drying power and diffusion of opacity.

The agent which I use to produce these effects is a hydrocarbon or mineral oil of the class obtained chiefly from the Texas, 35 Gulf and California oil fields. The oils in this class, or group, of which the "Texas oils" are regarded as the type, are known commercially as "asphaltic base oils," and are regarded chemically as being largely 40 composed of unsaturated hydrocarbons; and either the crude oil or any of its fractions, distillates or residuals, may be used in carrying out my invention. The specific oil which I have employed is that from the Sour Lake 45 district, Texas, preferably the available distillates now on the market, varying from .92 to .94 sp. gr. The specific gravity of the crude oil varies from .90 to .92 and that of the residuals from .990 to 1.000.

50. In carrying out my invention, I take the pigment desired for use, and grind it to paste form in one of the asphaltic-base-hydrocarbons. This compound, or magma, can be placed upon the market, like the present 55 form of pigment ground in oil, (which is

a mere matter of economical transportation) and, when desired for use as a paint, may be extended in any suitable oil-vehicle.

Instead, however, of thus grinding the pigment in the asphaltic base hydrocarbon and then adding the vehicle, the asphaltic base hydrocarbon may be incorporated in the selected vehicle, and the pigment ground in this mixture; the ultimate result being the same in either case.

The proportion of pigment used will depend upon its nature and may range, for example, from two hundred per cent. (200%) for chalk to three hundred per cent. (300%) for barytes, and to upward of six 60 hundred per cent. (600%) of sublimed compounds of zinc and lead. The percentage of asphaltic-base hydrocarbon to be incorporated in the vehicle will also vary with the nature of the pigment and the vehicle, from 65 eight to twelve per cent., or an average of ten per cent., giving good results in general.

Any fatty oil, such as linseed oil, may be employed as a vehicle, but very satisfactory and economical compositions can be 70 formed with the non-drying and semi-drying fatty oils, as in examples 4, 5, 6, 8 and 9, below given. The compositions, while possessing great spreading power and opacity, 75 may be slow in drying and I prefer, in all cases, to accelerate the drying action by incorporating another drying oil, preferably tung oil, or a mixture of tung oil and marine animal oil, the result being a very decided reduction in the time required for drying. 80 The use of tung oil in conjunction with the Texas oil is specifically claimed in application No. 443671, filed February 9, 1921.

85. As the asphaltic base hydrocarbons will act as solvents for many of the animal, vegetable and mineral residuals, waxes, resins, stearins, and the like, it may be found advantageous, in some cases, to incorporate a small proportion of one or more of these substances in the composition, as they will 90 render the ultimate paint-film much more resistant to atmospheric and abrasive influences. Thus, naphthalene ( $C_{10}H_8$ ) by reason of its great abundance, would be a 95 most economical agent to use, from three (3) to five (5) per cent., added to the oil-vehicle, or to the asphaltic base hydrocarbon, greatly increasing the permanency of the paint-film.

100. The asphaltic-base-hydrocarbon may, if desired, be oxidized or hydrogenated, or 105

110

both; and although the initial reaction in each case is feeble, yet sufficient molecular change is effected to increase its reaction when brought into contact with pigments and oil-vehicles, or oxidizable matter. A run of two (2) or three (3) hours on oxidizers at a temperature of 250° Fahr., and a run of half (½) or three-quarters (¾) of an hour, with hydrogen, in the presence of catalysts, will be sufficient.

The oxidation and hydrogenation of the hydrocarbons, are claimed in applications Nos. 443672 and 443673, filed February 9, 1921.

- 15 The term zinc-lead, as used herein, is intended to designate a class of pigments which have been on the market for many years and are now well-known in the trade by that name. They are all composed of 20 zinc oxid and lead sulfate in varying proportions, the one which I prefer consisting, approximately, of 60 per cent. zinc oxid and 40 per cent. lead sulfate.

The following are examples of compositions which will produce satisfactory results:

- (1) Eighty (80) parts linseed oil; ten (10%) per cent. asphaltic base hydrocarbon of .9302 sp. gr.; fifteen (15%) per cent. 30 tung-oil; one hundred fifty (150) parts barytes (natural); and thirty (30) parts zinc-lead (sixty (60%) per cent. zinc oxid and forty (40%) per cent. lead sulfate).
- (2) Eighty (80) parts linseed oil; fifteen (15%) per cent. asphaltic base hydrocarbon of .9302 sp. gr.; fifteen (15%) per cent. tung oil; fifteen (15%) per cent. menhaden oil; one hundred fifty (150) parts barytes (natural); and thirty (30) parts zinc lead.
- (3) Eighty (80) parts linseed oil; fifteen (15%) per cent. asphaltic base hydrocarbon, oxidized and hydrogenated, of .9370 sp. gr.; fifteen (15%) per cent. tung oil; and one hundred (100) parts zinc lead.
- (4) Eighty (80) parts soja oil; ten (10%) per cent. asphaltic base hydrocarbon, hydrogenated, of .9302 sp. gr.; fifteen (15%) per cent. tung oil; one hundred fifty (150) parts barytes; and thirty (30) parts zinc lead.
- (5) Eighty (80) parts cotton oil; ten (10%) per cent. asphaltic base hydrocarbon, hydrogenated, of .9302 sp. gr.; fifteen (15%) per cent. tung oil; fifteen (15%) per cent. menhaden oil; thirty (30) parts chalk; and thirty (30) parts zinc lead.
- (6) Eighty (80) parts cotton oil; ten (10%) per cent. asphaltic base hydrocarbon, hydrogenated, of .9302 sp. gr.; fifteen (15%) per cent. tung oil; one hundred fifty (150) parts barytes; and thirty (30) parts zinc lead.
- (7) Eighty (80) parts linseed oil; fifteen (15%) per cent. asphaltic base hydrocarbon, 65 of .9302 sp. gr.; fifteen (15%) per cent. tung

oil; fifteen (15%) per cent. menhaden oil; three (3%) per cent. naphthalene; one hundred fifty (150) parts barytes (natural); and thirty (30) parts zinc lead.

(8) Eighty (80) parts soja oil; ten (10%) per cent. asphaltic base hydrocarbon, hydrogenated, of .9302 sp. gr.; fifteen (15%) per cent. tung oil; five (5%) per cent. naphthalene; one hundred fifty (150) parts barytes (natural); and thirty (30) parts zinc lead.

(9) Eighty (80) parts soja oil; fifteen (15%) per cent. tung oil; fifteen (15%) per cent. menhaden oil; ten (10%) per cent. asphaltic base hydrocarbon, hydrogenated, showing .9302 sp. gr.; three (3%) per cent. naphthalene; thirty (30) parts powdered serpentine (as talc or asbestos); thirty (30) parts calcium silicate; and thirty (30) parts zinc-lead.

The above mixtures, with the usual quantity of commercial liquid drier added, when spread as a paint, will firm or dry in from two and one-half (2½) to five (5) hours, and subsequently indurate satisfactorily.

By means of my invention, all the so-called inert or inactive substances which, heretofore, have been used in the painter's art as mere adulterants, may be employed as a basis for paint, as the magma formed by 95 grinding such substances in the asphaltic-base-hydrocarbon, not only immediately becomes congruent to all oil-vehicles, but also assists, with its diffusive opacity, in increasing the index of refraction. Opacity is one 100 of the most expensive attributes of the present system of painting as based on the use of Dutch white lead, because so much more pigment is used than is necessary, that the result is a decided economic loss. When, however, all inert, or inactive matter, is brought into active participation in diffusive opacity, as is done by my invention, and a paint produced which will not deteriorate, the result is a decided economic gain. The 105 result obtained is very marked with barium sulfate, natural; the lead salts, such as the sulfate and carbonate, even in a minute crystalline condition; silica, and the silicious minerals in general, such as calcium and magnesium; and the serpentines, such as talc, asbestos, and the like.

Any suitable commercial liquid drier may be used. All the oil factors in the compounded oil-vehicle must, for the best effects, 120 be water free.

The paint composition made with the vehicle above described, is claimed in another application filed herewith and bearing the Serial Number 174,256.

I am aware that it has been proposed, heretofore, to use crude hydrocarbons, as well as the residuals of distillation, in admixture with a variety of other ingredients, for water-proofing and cement purposes, but 130

- such compositions I expressly disclaim, as they did not have for their object the formation of an anhydrous system of painting and could not be used for my purpose. I believe myself to be the first to employ the unsaturated hydrocarbons known commercially as asphaltic base hydrocarbons, in a paint-vehicle for the purpose of adapting it for successful use with the anhydrous pigments.
- 10 Having thus fully described my invention, I claim:—
1. A paint-vehicle comprising a fatty oil; and a mineral oil of the Texas oil type.
  2. A paint-vehicle comprising a fatty oil;
- a mineral oil of the Texas oil type; and 15 tung oil.
3. A paint-vehicle comprising a non-drying fatty oil; and a mineral oil of the Texas oil type.
  4. A paint-vehicle comprising a non-drying fatty oil; a mineral oil of the Texas oil type; and tung oil.
  5. A paint-vehicle comprising a fatty oil; a mineral oil of the Texas oil type; and an agent resistant to atmospheric and abrasive 25 influences.

WM. N. BLAKEMAN, JR.